

July 12, 1960

F. J. BOURBEAU ET AL

2,944,294

METHODS FOR TREATING POLYMERIC PLASTIC SURFACES

Filed July 1, 1957



*François J. Bourbeau  
John Steenhalgh  
and  
Claude J. Valler, Jr.*  
INVENTORS

*BY Brown and Mikulla  
and  
Herbert S. Kassman*

ATTORNEYS

1

2,944,294

## METHODS FOR TREATING POLYMERIC PLASTIC SURFACES

Francis J. Bourbeau, Randolph, John Greenhalgh, Wellesley, and Claude F. Valle, Jr., Waltham, Mass., assignors to Polaroid Corporation, Cambridge, Mass., a corporation of Delaware.

Filed July 1, 1957, Ser. No. 669,064

4 Claims. (Cl. 18—56)

This invention relates to improved methods for polishing polymeric plastic films to be used, for example, in connection with sheets intended to provide a base for a photographic image-carrying layer.

It has long been recognized that certain linear polymeric plastic materials, such, for example, as cellulose acetate, are useful in connection with the making of photographic prints. In the well-known Land diffusion-transfer process, for example, polymeric plastic materials, such as cellulose acetate, provide a highly satisfactory base layer for subsequent layers upon which silver is precipitated to form a positive photographic image. It is desirable, in connection with such processes, that uniformity and high gloss be imparted to that surface of such a polymeric plastic base layer to which such subsequent layers are applied.

To obtain these properties, it is customary to deposit a coating of cellulose acetate or a similar material upon one surface of a paper stock and then to polish the exposed surface of the coating; this is commonly done by bringing the coated stock into contact with a smooth, hard surface such, for example, as a chrome-plated drum. Conventionally, there are limits to the speed and ease of polishing such surfaces. For example, if a conventional procedure is followed whereby a thin coating of cellulose acetate is applied to the base paper and, after some solvents have been removed, the coating is polished for improved smoothness and gloss, satisfactory polishing will be obtained only if the partly dried coating comes in contact for a relatively long period with a heated, polished chrome drum. This requirement for extended contact necessarily reduces the rate at which coated stock may be polished; this may well be the bottleneck in an entire production operation.

Accordingly, the objects of the present invention are to provide methods for improving the gloss and uniformity of plastic sheets and coatings; to permit production of high-gloss coated stock at high speeds; and to provide a uniform, high-gloss base layer for receiving photographic images printed by means of the Land diffusion-transfer process.

Other objects of the invention will in part be obvious and will in part appear hereinafter.

The invention accordingly comprises the process involving the several steps and the relation and order of one or more of such steps with respect to each of the others which are exemplified in the following detailed disclosure, and the scope of the application of which will be indicated in the claims.

For a fuller understanding of the nature and objects of the invention, reference should be had to the following detailed description taken in connection with the accompanying drawing which is a schematic representation of a preferred apparatus for practicing the invention, showing also the arrangement of steps in the preferred process.

A preferred embodiment of the improved process herein described consists essentially in applying a coating of

2

a linear polymer, such as cellulose acetate, to a base paper such as baryta stock, drying the coating to remove as much of the solvent as is practicable, and feeding the coated stock to a smooth-surfaced polishing drum, simultaneously applying at the nip a minute quantity of a liquid, which has the property, in the quantity and duration of application, of softening but not completely dissolving the cellulose acetate coating. The liquid is preferably so selected that, in the amount applied and for 10 the interval during which it is in contact with the surface to be polished, at least the skin portion of the cellulose acetate layer is softened. Water, for example, may be employed as a softener for cellulose acetate, but since water has a relatively slow softening action, it is desirable to maintain the surface to be polished in contact with the polishing drum for a relatively longer period than would be desirable for a liquid which softens at a more rapid rate, such, for example, as a methanol-water mixture.

Referring now to the schematic representation in the drawing, the preferred apparatus may comprise a supply reel 1 upon which coated and dried stock has been wound, spatially separated from a parallel tension roller 2 which is in turn disposed directly below a nip roller 3. Nip roller 3 is preferably provided with a nonmetallic, slightly yieldable surface and may be so disposed as to press the stock against a polishing drum 14. Above the nip roller 3 is positioned reservoir 4, which is of any suitable configuration to hold a desired amount of the softening liquid. The base of reservoir 4 is provided 30 with an opening 5, leading to a manifold 6. A suitable feed control valve 8 may be provided in the line to manifold 6 or at any other point in the feed assembly. Manifold 6 may have a series of exit apertures each connecting with a feed tube 10 leading to the nip 12. Preferably, feed tubes 10 should be so spaced laterally that a small, continuous bead of liquid will form at the nip; a lateral spacing of the order of six inches is generally suitable.

Contacting nip roller 3 is a large polishing drum 14. Drum 14 preferably has a cylindrical, polished chrome-plated surface which is as free as possible from scratches, projections or other irregularities. Drum 14 may have provision for heating the polished surface from within by means, for example, of an annular jacket and suitable supply and return passages for passing hot water through the jacket. Provision may be made for varying the pressure of nip roller 3 against drum 14.

Directly adjacent to drum 14 is positioned tension roller 16, which is in turn spaced a suitable distance from an end storage reel 18.

The process is preferably performed in the following manner. Paper stock such as baryta paper is coated by any suitable means with a thin layer of cellulose acetate which may be applied in the form of a solution made up of cellulose acetate flake dissolved in suitable solvents. For example, a suitable solution may comprise 25 g. cellulose acetate, 180 cc. ethyl acetate and 60 cc. methanol. The coated stock is then dried to remove as much of the solvents as feasible, preferably until less than the order of 5% of the original solvent remains. Preferably, the stock should be dry enough to be rollable without blocking. The coated stock may then be wound on a suitable core which may then be positioned as supply reel 1. From reel 1, the coated and dried stock preferably passes under tension roller 2, around nip roller 3 and is pressed into contact with drum 14. A minute quantity of a liquid is applied to the coated surface just as it comes into contact with drum 14. This liquid, supplied from reservoir 4 through manifold 6 and feed tubes 10, preferably comprises a mixture of 80% methanol and 20% water, by weight. The methanol-water mixture may preferably be regulated so that two to three drops per second are applied

from each feed tube 10. The rate of flow should be such that only a small, continuous bead of water-methanol can be seen at the nip. The coated stock is then maintained in contact with the polishing drum 14 for a time on the order of one second. The drum surface may preferably be at a temperature of about 180° F., although temperatures on the order of 30 to 40° higher and 50 to 60° lower do not lead to significantly different results. The pressure of the stock against the drum 14 is not critical, so long as at least a minimal pressure is maintained; a good polish will result at pressures ranging from 10 to 250 pounds per linear inch of stock width, or at even higher pressures.

The stock is stripped from drum 14 by means of tension roller 16 and may then be wound around storage reel 18 for further processing.

Tests have indicated that baryta paper coated with cellulose acetate and treated on the apparatus and in accordance with the process described above may be polished to a high, uniform gloss at speeds of the order of 100 linear feet per minute. Conversely, slower speeds yield an unusually high uniform gloss.

Several alternative arrangements and procedures are possible without departing from the scope of the invention. For example, it is to be understood that the process described above may be incorporated with other earlier and later processes in an assembly line technique by eliminating reels 1 and 18 and instead feeding the stock continuously from or to other equipment.

The apparatus may also be varied by replacing reservoir 4 and its associated feeding system with suitable devices for spraying or otherwise depositing the water-methanol mix upon the cellulose acetate coating at the nip.

Polishing drum 14 may have any suitable internal heating arrangement or may be heated externally. As has been previously indicated, the drum surface temperature may be varied widely. Preferably, the temperature need only be high enough to assist in softening the surface to be polished and to cause substantial redrying of that surface before it is separated from the drum surface. The upper temperature limit is similarly flexible; the drum temperature should not be so high as to cause the softening liquid to boil away before it has performed its softening function, nor should the temperature be high enough to cause the plastic surface to become overly tacky or to develop other unfavorable properties. The drum surface may be chromium or a chrome alloy, stainless steel, glass, or any other material that will impart the desired surface characteristics to the stock. Although it has been found convenient to use a polishing drum having a diameter between 3 and 6 feet, larger or smaller drums may be used.

A wide variety of materials may be used in the process. For example, other papers or cloths may be used as the base material instead of baryta paper, or one surface of a preformed plastic film may be polished in this manner. Any thermoplastic material which may be softened by a suitable selection of softening agents and heating conditions may be employed. For example, ethyl cellulose or polyvinyl chloride may similarly be polished.

Similarly, a great number of surface-softening materials may be used instead of the water-alcohol mixture. Water, methanol, ethanol and butanol may be used with cellulose acetate at relatively low processing speeds; mixtures of water and other compounds, such as ethanol-water, propanol-water or an acetone-water mixture will be effective even at higher processing speeds, i.e., on the order of 100 feet per minute, as will ternary mixtures, such as equal proportions, by weight, of water, methanol and ethyl acetate. In general, it is desirable to use materials or mixtures in which the polymeric plastic to be polished is only slightly soluble, i.e., those materials which may be classed as swelling agents for the polymer within the period of application of the material to the surface. The term "swelling agent" as used herein shall be understood to in-

clude solvents as well as substances which swell or soften the polymeric plastic to which they are applied without actually dissolving it.

It is probable that the increased polishing rate permitted by the present invention is based on the following phenomena:

In conventional polishing, it is customary to apply the coated stock to a large-diameter, slowly-rotating polishing drum while a substantial percentage of solvent remains in the coating. In this condition, the coating must remain in contact with the drum for a relatively long period of time to cause the entire coating thickness to be hardened. In the present invention, the coating is fully dried and hardened beforehand. The subsequent application of the softening agent at the nip probably penetrates and softens only an extremely thin skin of the coating. Thus, this small skin may be smoothed and dried to a high polish during a relatively short contact with the polishing drum. As a result, a high gloss may be obtained at significantly higher linear speeds.

Although a prime object of the present invention is to provide an optically smooth, high-gloss surface upon a polymeric plastic material, it is obvious that other surface characteristics may be imparted by substituting, for the smooth polishing drum of the preferred embodiment, a surface having other characteristics such as, for example, lenticules or a pebble, wrinkle, or sand finish. The terms "polishing element" and "polishing surface" as used herein shall be understood as including not only smooth surfaced elements but also those having the other indicated surface characteristics.

Since certain changes may be made in the above process without departing from the scope of the invention herein involved, it is intended that all matter contained in the above description or shown in the accompanying drawing shall be interpreted as illustrative and not in a limiting sense.

#### What is claimed is:

1. The method of polishing the surface of a substantially solvent-free, hardened thermoplastic polymeric layer carried upon a paper support to a high gloss which comprises the steps of providing at least one source of a softening agent for said polymeric layer, moving said polymeric layer past said source of softening agent, contacting said polymeric layer during movement past said source with a quantity of softening agent sufficient to soften only a thin surface portion of said polymeric layer, substantially immediately after passing said source pressing the softened layer surface into contact with a rotating smooth-surfaced polishing element, said polishing element being heated to a temperature sufficient to substantially redry said softened layer surface, and maintaining said softened layer surface in contact with said heated, rotating polishing element until a smooth, hard, high-gloss surface is formed.

2. The method of claim 1 wherein said support is baryta paper and said polymeric layer is cellulose acetate.

3. The method of claim 1 wherein said softening agent comprises a solution of water and alcohol.

4. The method of claim 3 wherein said softening agent comprises a solution of about 80 percent by weight of methanol and about 20 percent by weight of water.

#### References Cited in the file of this patent

#### UNITED STATES PATENTS

|           |               |                |
|-----------|---------------|----------------|
| 1,860,456 | Dreyfus       | May 31, 1932   |
| 1,889,045 | Dreyfus       | Nov. 29, 1932  |
| 1,889,061 | Dickie et al. | Nov. 29, 1932  |
| 1,912,625 | Dreyfus       | June 6, 1933   |
| 1,964,724 | Dreyfus       | July 3, 1934   |
| 2,218,227 | Winnek        | Oct. 15, 1940  |
| 2,296,804 | Winnek        | Sept. 22, 1942 |
| 2,562,078 | Winnek        | July 24, 1951  |